

## UNITED STATES PATENT OFFICE

VERE B. BROWNE, OF BRACKENRIDGE, PENNSYLVANIA

## METHOD OF PRODUCING MAGNETIC ALLOYS

No Drawing.

Application filed February 20, 1930. Serial No. 430,140.

This invention relates to a method of manufacturing silicon steel for use as a magnetic alloy.

Silicon steel is now largely used as a magnetic alloy in the manufacture of certain parts of electrical apparatus on account of its high degree of magnetic permeability, and low degree of magnetic hysteresis, and this invention has particularly to do with the manufacture of silicon steel for use as a magnetic alloy.

An object of the invention is to produce a silicon steel alloy having a higher degree of magnetic permeability than such alloys at present known and used for this purpose.

A further object of the invention is to provide a silicon steel alloy for use as a magnetic material in electrical apparatus, having a low carbon content, and that will be practically free from dissolved gases.

A further object of the invention is to provide a method by which silicon steel alloys having a high degree of magnetic permeability, and which are free from dissolved gases, may be manufactured.

Other objects of the invention will be apparent to those skilled in the art.

Silicon steel, (also known as silicon iron) has been known for some time as a valuable iron alloy for use in electrical apparatus. Its value is not only determined by its silicon content, but by its soundness and purity as well. Recent research on these alloys has shown that carbon plays an important part in the value of such material, and it has now been found that the presence of dissolved or occluded gases also plays an important part in the value of the alloys for use in the magnetic circuits of electrical apparatus.

Small laboratory quantities of silicon steel having an extremely low carbon content have been produced in a vacuum furnace, but by methods which are wholly impracticable for commercial production on a large scale.

In my prior United States patents, Numbers 1,570,229, dated January 19, 1926, and 1,574,550, dated February 23, 1926, are disclosed methods of producing silicon steel alloys for use in electrical apparatus. In each of these patents the final operation is

the tapping of the low carbon iron in the molten condition into a ladle containing ferro silicon sufficient to bring the alloy up to the desired composition. When the iron is raised to a high temperature as described in said 55 patents, especially when currents of air are passed through the metal, the melted iron dissolves a large volume of gases. When silicon is added to the molten iron, it has been found that the silicon increases the solubility of the iron for the gases contained 60 therein, with the result that all of the gases which were originally held in solution on account of the high temperature of the metal are retained in the final product. The gases 65 blown through the molten metal, and other gases which may have been absorbed in the process of making the iron, include some carbon monoxide and carbon dioxide, with the result that the final product will show a 70 greater carbon content than exists therein in the form of iron carbide; in addition to the above gases, other gases such as nitrogen and hydrogen are frequently present. The presence of the dissolved gases is disadvantageous 75 in this type of alloy, since it has been found that they produce a detrimental effect on the magnetic properties of the final product.

In the present invention, the product of 80 the Bessemer, or open hearth, or electric furnace, as described in the above patents, which product is an iron free from silicon, and having a carbon content of not over 0.03 percent, is subdivided by casting into suitable 85 sized ingots which are permitted to solidify so that the gases which are dissolved or occluded therein are allowed to escape during the solidification and the lowering of their temperature to the atmospheric temperature. 90 The cooled ingots, which are now free from the dissolved or occluded gases, may then be rolled and cut up into suitable sizes for final charging into an electric induction furnace; or instead of casting the metal into ingots, 95 it may be cast into small moulds to make slabs of a suitable size for charging into the induction furnace direct, or the melted metal may be shotted by being cooled rapidly in water. The solid metal is then charged into 100

the induction furnace and melted, with the necessary ferro silicon or other source of silicon to produce a desired composition in the final product, or the ferro silicon or the like <sup>8</sup> may be added after the iron is melted. By these methods I am able to produce a silicon steel alloy having a carbon content of less than 0.03 percent, and containing the desired quantity of silicon, and which is substantially free from dissolved gases.

<sup>10</sup> The silicon steel alloy produced by the methods described herein, may now be manufactured into suitable sheets for transformer cores, or cast into suitably shaped magnetic <sup>15</sup> frames; the alloy has a higher degree of magnetic permeability, and a lower magnetic hysteresis loss, than is found in silicon steel alloys heretofore produced.

I claim:

<sup>20</sup> 1. A method of producing magnetic alloys including suitably producing a molten body of low carbon iron substantially silicon-free, casting the same into suitable ingots, whereby the molten body solidifies and is cooled to <sup>25</sup> atmospheric conditions, thereby expelling gases therefrom, rolling said ingots, further subdividing them, and remelting the same while simultaneously adjusting the silicon content to the desired amount by suitable <sup>30</sup> additions to the remelted mass.

<sup>35</sup> 2. A method of producing magnetic silicon alloys of high magnetic permeability including preparing a molten body of low carbon iron which is substantially silicon free and which contains not over about 0.03% carbon, subdividing the molten mass into smaller parts, cooling and solidifying the subdivided parts to about atmospheric conditions until they expel their gases therefrom <sup>40</sup> and remelting the same while adjusting the silicon content by predetermined additions to the remelted mass.

In testimony whereof, I have hereunto subscribed my name this 17th day of February, <sup>45</sup> 1930.

VERE B. BROWNE.